

O. WOODWARD.

PROCESS OF MAKING TYPE BLOCKS FOR TYPE WRITING AND LIKE MACHINES.  
APPLICATION FILED MAY 6, 1911.

1,115,643.

Patented Nov. 3, 1914.

FIG.5.



FIG.4.



FIG.3.



FIG.2.



FIG.1.



FIG.11.



FIG.10.



FIG.9.



FIG.6.



FIG.8.



WITNESSES:

*E. M. Wells*  
*Marie E. Smith*

INVENTOR:

*Oscar Woodward*  
*By Jacob Field*

HIS ATTORNEY

# UNITED STATES PATENT OFFICE.

OSCAR WOODWARD, OF MONTCLAIR, NEW JERSEY, ASSIGNOR, BY MESNE ASSIGNMENTS, TO REMINGTON TYPEWRITER COMPANY, OF ILION, NEW YORK, A CORPORATION OF NEW YORK.

## PROCESS OF MAKING TYPE-BLOCKS FOR TYPE-WRITING AND LIKE MACHINES.

1,115,643.

Specification of Letters Patent.

Patented Nov. 3, 1914.

Application filed May 6, 1911. Serial No. 625,496.

To all whom it may concern:

Be it known that I, OSCAR WOODWARD, citizen of the United States, and resident of Montclair, in the county of Essex and State 5 of New Jersey, have invented certain new and useful Processes of Making Type-Blocks for Type-Writing and like Machines, of which the following is a specification.

My invention relates to the process of 10 making type blocks for typewriting and like machines.

Heretofore it has been customary to provide type blocks with integral shanks by which the blocks could be attached to the 15 type bars. In some instances these blocks and shanks were hardened to a like degree throughout in order to provide hard type faces that could not be easily defaced or injured. In such constructions, however, it 20 was found that the shanks could not be easily bent in order to afford an adjustment of the block on the bar as is often required to place the type "on its feet" or for properly aligning the type. In some cases the type blocks 25 and their shanks were made of comparatively soft metal in order to facilitate this adjustment of the type blocks, but this proved to be disadvantageous since it resulted in the type faces being easily defaced or injured.

The main object of my invention is to 30 overcome the above and other disadvantages and to provide an improved process for making a type block having a hardened type face and a relatively soft shank, so that the shank 35 may be easily bent to afford an adjustment of the type block on the bar and yet provide a hard type face, and one which is not easily injured or defaced.

A further object of my invention is to 40 provide a comparatively simple, inexpensive and efficient process by which the small type blocks with hard type faces and relatively soft integral shanks may be produced in large quantities.

To the above and other ends which will 45 hereinafter appear, my invention consists of the process of making type blocks to be hereinafter described and particularly pointed out in the appended claims.

In the drawings wherein like reference 50 characters indicate corresponding parts in the different views, Figure 1 is a perspective view of a blank stamped out of sheet metal

and from which the type block and its integral shank is made. Fig. 2 is a like view 55 of the same after it has been tumbled and the sharp corners and edges have been removed. Fig. 3 is a perspective view of the blank after it has been pressed to flatten it. Fig. 4 is a like view of the blank after the 60 shank has been turned. Fig. 5 is a perspective view of the blank after it has been submitted to pack-annealing. Fig. 6 is a like view of the blank after it has been nickel plated. Fig. 7 is a perspective view of the 65 blank after the face of the nickel plated blank has been milled off. Fig. 8 is a perspective view, looking toward the face of the type block, after the types have been formed thereon. Fig. 9 is a bottom perspective view 70 of the same. Fig. 10 is a perspective view of the type block after the sides thereof have been ground off. Fig. 11 is a like view of the finished type block.

The type blocks are first formed in blanks 75 such as that represented in Fig. 1 by stamping the blanks out of sheet metal of mild or soft steel. Each blank, as will be seen, comprises a body portion 1 which constitutes a type block proper and an integral shank 2 by 80 which the type block is to be connected to its type bar or carrier.

In the accompanying drawings I have 85 shown the blanks at different stages in the process of manufacture, beginning with the blank shown in Fig. 1 as it is first formed and ending with the completed type block shown in Fig. 11, ready for connection to its type bar. The blanks, formed as represented in Fig. 1, are then tumbled to remove the 90 sharp corners and edges thereof, thus leaving them as represented in Fig. 2. The act of punching out the blanks leaves them slightly bowed as indicated in Figs. 1 and 2 and after the blanks have been tumbled they 95 are pressed on the sides thereof between flat faces to flatten the blanks, as represented in Fig. 3. The blanks next have their shanks 2 turned as represented in Fig. 4 on an automatic machine employed for this purpose, 100 so that a shank of frusto-conical form is provided for its reception in a corresponding opening in the type bar.

After the shanks have been turned, as 105 represented in Fig. 4, they are inspected and any imperfect ones are thrown out. The

various steps to which the blanks are subjected thus far, such for instance as the punching and flattening steps, have a tendency to slightly harden the blanks and it is desirable that the blanks be rendered softer preliminary to the formation of the type faces thereon. The next step in the process, therefore, preferably consists in subjecting the blanks to pack-annealing. 10 The pack-annealing is effective to soften the metal by heating it and an additional amount of carbon is at the same time incorporated in the blank in order that parts thereof may be subsequently effectively hardened, as will hereinafter more clearly appear. If the character of the stock from which the blanks are made is such that it contains the requisite amount of carbon and also is sufficiently soft after having been 15 treated in the manner described preliminary to the formation of the type face, so that the type face may be properly formed thereon, then the step of pack-annealing may be omitted. In practice, however, I 20 prefer to employ the annealing step since it is difficult to obtain metal having the requisites referred to above. After pack-annealing, the blanks are plated, coated or covered with suitable material as for example 25 with nickel plating, as is intended to be represented in Fig. 6; the nickel plating covering every surface of the type block and its integral shank. After nickel plating the blanks, each blank has its face 6 milled off, 30 as represented in Fig. 7. In this view and others the parallel hatch lines are intended to represent the exposed metal from which the type block and its shank are formed, whereas the unshaded portions are intended 35 40 to represent the nickel plating. The blanks with their faces milled, as represented in Fig. 7, are then submitted to a cold pressing process by which the raised type faces 3 are formed. These type faces are formed in 45 the ordinary or any desired manner, such for example as in the manner disclosed in the patent to L. A. Diss No. 923,252, dated June 1, 1909. In the act of forming the type faces the metal is spread to form a bur 50 or flash 4 on all sides of the type block. This bur is afterward removed by grinding the sides of the type block, as represented in Fig. 10. After the bur or flash is removed the sides 5 of the type block, as 55 well as the face 6 thereof and the raised type faces 3, will have the body of the metal from which the type block is formed exposed, whereas the underside 7 and the shank 2 of the type block will be covered 60 with nickel plating. After each of the blocks has its sides ground in the manner shown in Fig. 10, the blocks are subjected to cementation, by first coating the blocks with what I term a cementing material, 65 such for example as cyanid of potassium.

While I have referred to the use of cyanid of potassium it should be understood that any suitable so-called cementing material may be used that will affect the exposed parts of the metal and will not affect the parts of the block that are covered, coated or plated with nickel or other suitable material. The blocks after being coated with a cementing material are heated and then quenched to harden only so much of each type block as has the nickel plating removed therefrom and where the body of the metal from which the type block is formed has been exposed to the action of the cementing material, as represented in Fig. 10. It follows, therefore, that the hardening by cementation in the manner described is effective only on the sides 5, the face 6 and the type faces 3 of the type-block, whereas the shank which is covered with a protecting coat of nickel plate remains comparatively soft and may be easily bent in order to afford an adjustment of the type block relatively to the type bar which carries it. The type faces and the body portion of the block being thus hardened, there is little liability of the type faces being defaced or injured. While a mere case hardening is preferred the depth of the action of the cementing material on the exposed portion of each type block will of course depend on circumstances and from certain aspects of the present invention it is immaterial to what depth the hardness extends in the block so long as the type face is hard and the stem relatively soft.

After the type blocks have been hardened in the manner described, they are, or may be, again nickel plated over their entire surfaces, as represented in Fig. 11, which shows the type block in completed condition.

It will be understood that I have provided a simple and efficient process of producing type blocks with hardened type faces and comparatively soft shanks by which they may be connected to the type bars or carriers, and which soft shanks afford an easy adjustment of the blocks by bending the shanks.

It is desirable to remove the face of the type block by milling it in the manner indicated in Fig. 7 in order that the raised type faces may be more clearly defined on the type block. It is likewise desirable to remove the bur 4 from the type block in order to present it in a finished manner. These two desirable steps in the process of manufacture are taken advantage of to remove parts of the nickel plating previously applied to the blank in order to expose to the action of the cyanid of potassium or other cementing material only those portions of the type block which it is desired to case harden. It will also be understood that in accordance with my present invention the small type blocks may be hardened

on their type faces in bulk; that separate handling is unnecessary and that a simple, inexpensive and efficient process is provided.

While I have described with considerable detail the various steps employed in the process of manufacturing type blocks in accordance with my present invention, it should be understood that various changes may be made in the process without departing from the invention as defined in the claims.

What I claim as new and desire to secure by Letters Patent, is:—

1. The process of making type blocks for the type bars of typewriting machines, this process consisting in forming plain-faced blocks, each being a single piece of unhardened metal, then converting those blocks into type blocks having plated shanks and unplated printing faces, and then treating the blocks with cementation-material and heating and cooling them.

2. The process of making type blocks for the type bars of typewriting machines, the process consisting in forming plain-faced blocks, each being a single piece of unhardened metal, then plating the blocks, then milling off their faces, then forming type on the milled faces by pressing the metal cold, then grinding off the burs formed on the blocks by the pressing operation, and then applying cementation-material to the blocks and heating and cooling them.

3. The process of making type blocks for the type bars of typewriting machines, this process consisting in forming from unhardened metal, blocks having type on their faces and plated shanks thin enough to enable them to be bent readily, and then coating the partly plated blocks with cementation-material and heating and cooling them.

4. The process of making type blocks for the type bars of typewriting machines, this process consisting in forming plain-faced blocks, each composed of a single piece of unhardened metal and comprising a body and shank, then converting these blocks into type blocks having type on their faces and plated shanks thin enough to enable them to be bent readily, and then coating the partly plated blocks with cementation-material and heating and cooling them.

5. The process of making type blocks for the type bars of typewriting machines, this

process consisting in forming plain-faced blocks, each composed of a single piece of unhardened metal and comprising a body and a shank thin enough to enable it to be bent readily, then entirely plating these blocks, then removing the plating that covers their faces, then forming type on their faces, and then coating the partly plated blocks with cementation-material and heating and cooling them.

6. The process of making type blocks for the type bars of typewriting machines, this process consisting in forming plain-faced blocks, each composed of a single piece of unhardened metal and comprising a body and a shank thin enough to enable it to be bent readily, then pack-annealing these blocks, then entirely plating them, then removing the plating that covers their faces, then forming type on their faces, and then coating the partly plated blocks with cementation-material and heating and cooling them.

7. The process of making type blocks for the type bars of typewriting machines, this process consisting in forming plain-faced blocks, each composed of a single piece of unhardened metal and comprising a body and a shank thin enough to enable it to be bent readily, then entirely plating these blocks, then removing the plating that covers their faces, then forming type on their faces, and then applying cyanid of potassium to these blocks and heating and quenching them.

8. The process of making type blocks for the type bars of typewriting machines, the process consisting in forming plain-faced blocks, each being a single piece of unhardened metal, then entirely plating the blocks with suitable material, then removing the plating from and forming type on the faces of the blocks, and then coating the partly plated blocks with cementation-material and heating and cooling them.

Signed at the borough of Manhattan, city of New York, in the county of New York, and State of New York, this 5th day of May, A. D. 1911.

OSCAR WOODWARD.

Witnesses:

CHARLES E. SMITH,  
E. M. WELLS.